

R. J. SHOEMAKER,  
METHOD OF PLATING METAL ARTICLES.  
APPLICATION FILED MAR. 5, 1918.

1,330,399.

Patented Feb. 10, 1920.



Witnesses:

W. F. Kilroy

Harry C. White

Robert J. Shoemaker  
Inventor  
By, *Barney Freeman*  
Attest.

# UNITED STATES PATENT OFFICE.

ROBERT JAY SHOEMAKER, OF MILWAUKEE, WISCONSIN.

## METHOD OF PLATING METAL ARTICLES.

1,330,399.

Specification of Letters Patent. Patented Feb. 10, 1920.

Application filed March 5, 1918. Serial No. 220,419.

*To all whom it may concern:*

Be it known that I, ROBERT J. SHOEMAKER, a citizen of the United States, residing at Milwaukee, in the county of Milwaukee and State of Wisconsin, have invented certain new and useful Improvements in Methods of Plating Metal Articles, of which the following is a specification.

My invention relates to the art of plating metal articles, and has for a principal object to provide an improved method whereby this operation can be performed more expeditiously, economically and effectively than has been possible heretofore.

15 A further object is to provide a flux of novel composition for use in operations of this character.

The present invention is a development of the method described in the patent to McClintock and Shoemaker, No. 1,195,376, dated August 22, 1916, and in my co-pending application Serial No. 178,728, filed July 5, 1917.

20 The accompanying drawing shows diagrammatically an apparatus suitable for carrying out my improved method in connection with the plating of sheet metal with lead or other plating metal. The invention, however, is not limited to this treatment of 25 sheet metal, but may be utilized for so treating pipes, boiler flues, or other articles.

25 Referring to the drawings, A designates a vat in which the metal sheets are pickled in acid, muriatic acid, for example, before being brought into contact with the plating metal. B is a furnace having a retort C to contain a body D of plating metal, for example, lead, or some of the common alloys of lead. The sheet of metal E is taken 30 from the pickling vat and run between rollers F, F, arranged so that the acid squeezed from the plate by the rolls will run back into vat A. G is a frame arranged at the surface of the body of molten plating metal D containing a body of flux H which floats on the plating metal. The rest of the surface of the body of plating metal is preferably covered with a thin film of the flux I, the purpose of which is to prevent oxidation of the 35 molten metal as described in my application Serial No. 178,728, above mentioned. The metal sheet passes through the body of flux on the frame G into the molten plating metal, and is withdrawn from the retort by 40 rollers J, J, and deposited on a conveyer K, or otherwise disposed of as convenience may

dictate; the sheet being preferably guided in its movement through the plating bath by guides L, M. The rollers J, J remove excess of the plating metal and make it certain that the plating metal is laid smoothly and evenly over the entire surface treated. This operation is facilitated by throwing powdered ammoniac occasionally on the rollers to keep them from scaling.

45 The flux which I use is composed of three metal chlorids, one of which is the chlorid of an alkaline metal. I prefer a composition consisting of zinc chlorid, common salt, and a small percentage of tin chlorid. The 50 preferred proportions by weight are eighty per cent. zinc chlorid, fifteen per cent. common salt (sodium chlorid) and five per cent. tin chlorid. I have found that the use of the tin chlorid as an ingredient of this flux 55 makes the plating metal flow much more readily over the surface of the article being plated than where the flux consists of zinc chlorid alone, or of zinc chlorid and common salt. Common salt is used with the 60 zinc chlorid to lower the melting point of the flux, as described in my pending application above mentioned.

65 By means of the improvement above described, it is possible to surface metal articles, such as steel or iron sheets, with a plating of lead or lead alloy (the term "lead" being intended to cover the common alloys of lead) which will permanently adhere to the sheet and will uniformly cover the entire surface treated without pin holes, or other imperfections. I prefer to use, as a metal for lead plating, an alloy consisting substantially of eighty-five per cent. of lead, ten per cent. of antimony and five per cent. of tin.

70 I claim:

1. A flux for plating operations containing zinc chlorid as a principal ingredient together with tin chlorid.
2. A flux for plating operations containing zinc chlorid as a principal ingredient together with tin chlorid and common salt.
3. A flux for plating operations composed of approximately eighty per cent. of zinc chlorid, five per cent. of tin chlorid and fifteen per cent. of common salt.
4. Improvement in the art of plating metal articles which consists in passing the article through a molten flux consisting of zinc chlorid as a principal ingredient together with tin chlorid and common salt,

and thereafter submerging the article in a bath of molten plating metal.

5. Improvement in the art of plating iron or steel articles with lead which consists in passing the article through a molten flux consisting of zinc chlorid as a principal ingredient together with tin chlorid and common salt, and thereafter submerging the article in a bath of molten plating metal.
- 10 6. Improvement in the art of plating iron or steel articles with lead, which consists in

passing the article through a molten flux consisting of zinc chlorid as a principal ingredient together with tin chlorid and common salt, which is supernatant on a bath of the plating metal, and thereafter causing the article to be submerged in the plating metal bath.

7. A flux for plating operations composed of a mixture of three metallic chlorids, one of which is the chlorid of an alkaline metal.

ROBERT JAY SHOEMAKER.